

# UNITED STATES PATENT OFFICE.

ANTON G. CHRISTMAN AND CHARLES W. KOEPP, OF MILWAUKEE, WISCONSIN.

## PAINT COMPOSITION.

1,342,497.

Specification of Letters Patent.

Patented June 8, 1920.

No Drawing.

Application filed January 17, 1920. Serial No. 352,190.

*To all whom it may concern:*

Be it known that we, ANTON G. CHRISTMAN and CHARLES W. KOEPP, both citizens of the United States, and residents of Milwaukee, in the county of Milwaukee and State of Wisconsin, have invented certain new and useful Improvements in Paint Compositions; and we do hereby declare that the following is a full, clear, and exact 10 description thereof.

Our invention relates to new and useful improvements in paint compositions for producing a simple, economical and durable finish for wood, metal or other surfaces.

15 A further object of our invention is to provide a paint composition for producing a "flat" finish.

With the above and other objects and advantages in view, our invention resides in 20 the novel combination of ingredients hereinafter more fully described.

Our paint includes a vehicle consisting of a mixture of a powdered or granulated mineral, turpentine, linseed oil, a mineral 25 oil, such as purified benzin, and a drier, such as Japan or varnish; and a pigment consisting of a solution of glue, borax, sal soda and sugar of lead in water.

In preparing the paint we prefer to use 30 the ingredients in the following proportions—for the vehicle: four ounces to one-half pound of a powdered or granulated mineral, one quart of turpentine, one quart of linseed oil, one and one-half quarts of 35 mineral oil, and one-half pint of a drier;

for the pigment: a solution in water of substantially—ten ounces of glue; twelve ounces of borax, twelve ounces of sal soda, and twenty ounces of sugar of lead. A half pint of this solution is added to the vehicle. 40

The proportions given are those for a gallon of the paint.

The paint is applied to the surface to be covered in the ordinary manner and produces a durable and economical "flat" finish. 45

I claim:

1. A paint composition comprising a vehicle containing the following ingredients: powdered mineral, turpentine, linseed oil, mineral oil and a drier, and a water solution 50 of the following ingredients: glue, borax, sal soda, and sugar of lead.

2. A paint composition comprising a vehicle containing the following materials in substantially the following proportions: 55 four to eight ounces of a powdered mineral, one quart of turpentine, one quart of linseed oil, one and one-half quarts of a mineral oil, one-half pint of a drier; and a half pint of a water solution of the following materials in substantially the following proportions: ten ounces of glue, twelve ounces of borax, twelve ounces of sal soda, and twenty ounces of sugar of lead. 60

In testimony that we claim the foregoing 65 we have hereunto set our hands at Milwaukee, in the county of Milwaukee and State of Wisconsin.

ANTON G. CHRISTMAN.  
CHAS. W. KOEPP.